

1

2,861,952

## DECOLORIZATION OF LUBRICATING OILS

William E. Thompson, Wallingford, and Robert W. Shinn, Swarthmore, Pa., assignors to Sun Oil Company, Philadelphia, Pa., a corporation of New Jersey

No Drawing. Application January 25, 1957  
Serial No. 636,251

3 Claims. (Cl. 252—50)

This invention relates to a process for decolorizing lubricating oils, and more particularly to a process for decolorizing oils by exposure to visible light.

Hydrocarbon lubricating oils, particularly naphthenic oils prepared by distillation of essentially wax-free crude oils, contain small amounts of complex compounds which impart a dark color to the oil. While the presence of these compounds does not adversely affect the lubricating qualities of the oil, such oils are difficult to sell because customers prefer light-colored oils.

We have now discovered that stable, light-colored oils may be produced by exposing the oil to visible light at a temperature below about 40° F., followed by the incorporation of an antioxidant in the oil prior to bringing the oil to ambient temperatures. Exposure to visible light at room temperature has apparently no effect on the color of the oil, and ultraviolet light, even at low temperatures, also has no beneficial effect. The reason why light is effective at low temperatures, but not at room temperature is unknown to us, but it is speculated that at the higher temperatures, oxidation of oil components to dark colored compounds proceeds at a rate equal to the rate of removal of other colored compounds by light, so that there is no effect. The compounds destroyed by light are apparently natural oxidation inhibitors, since it has been observed that when irradiated oils are brought to room temperature without further treatment they tend to darken rapidly, and they cannot thereafter be lightened in color by further irradiation at reduced temperatures. If, however, an antioxidant such as phenylene diamine, diteriarybutyl paracresol, or any other petroleum anti-oxidant known to the art is added to the oil in the amount of from about .0005 to .005% before bringing it to room temperature the oil will remain stable in storage.

In order that those skilled in the art may more fully appreciate the nature of our invention and the method of carrying it out, the following examples are given.

### Example I

A quart bottle of a naphthenic lubricating oil having an O. D. color of 24.2 was placed on the laboratory roof during December, when the average temperature was under 40° F., and was below freezing most of the time. After 5 days' exposure, the color had been reduced to 15.9. The sample was then taken into the laboratory and held at room temperature for one day, after which its color had increased to 16.8. The bottle was then replaced on the roof. After an additional 6 days' exposure, the color had risen to 22.5. This indicates that natural antioxidants in the oil had been removed by the initial 5 days' exposure, and that oxidation,

2

once started, was autocatalytic, so that further exposure to light did not effect any decolorization.

### Example II

5 A duplicate sample was placed on the roof at the same time as the first sample and was left there, without warming, for 12 days, after which time it was found that it had dropped from its original O. D. color of 24.2 to an O. D. color of 13.5. Addition of 0.002% of diteriarybutyl paracresol to this oil, before warming to room 10 temperature, produced a stable oil which did not discolor in storage.

### Example III

15 A third duplicate sample was placed in a patch of snow on the roof. After only 5 hours in the sunlight the color was reduced from the original 24.2 to 17.1. Apparently this sample received a much greater dose of radiation than the samples of Examples I and II, due to reflection from the snow.

### Example IV

20 A fourth duplicate sample bottle was wrapped in tin foil so as to exclude light therefrom and was placed on the roof with the samples of the preceding examples. 25 After 8 days it was found that the color had increased to 24.9 from the original 24.2, indicating that cold alone was ineffective to decolorize the oil.

### Example V

30 A fifth duplicate sample was irradiated by ultraviolet light for six hours at 20° F. This treatment increased the O. D. color from 24.2 to 25.9, indicating that light in the visible spectrum was responsible for the decrease in color noted in the first three examples.

### Example VI

35 A quart bottle of a lubricating oil having an initial O. D. color of 20.1 was placed on the roof and exposed for 70 days during the winter. It had a final color of 10.6, and could be stabilized at this color by the addition of 0.002% of phenylene diamine. A similar bottle placed in sunlight on the laboratory window sill during the same period of time was reduced in color only from 20.1 to 19.8, indicating that irradiation by light at room 40 temperature is ineffective in reducing color.

### Example VII

45 A quart bottle of a different lubricating oil having an initial O. D. color of 18.4 was placed on the roof in December and kept there for six days, after which the color was found to be 12.4. A duplicate bottle kept on the laboratory shelf increased in color during the same period to 21.0.

### Example VIII

55 A quart bottle of a still different lubricating oil having an initial O. D. color of 13.8 was placed on the roof at the same time as the bottle of Example VII. After six days, the color of this oil had decreased to 10.4 while a duplicate kept on the laboratory shelf retained its original color over the same period of time.

We claim:

1. A process for decolorizing lubricating oils which comprises bringing a petroleum lubricating oil prepared by distillation of an essentially wax-free naphthenic crude oil and containing naturally occurring impurities in an

amount sufficient to impart a dark color to the oil to a temperature less than about 40° F., irradiating the oil with light in the visible spectrum for a period of time sufficient to effect a reduction in the O. D. color of the oil, and adding from about 0.0005% to about 0.005% of an antioxidant selected from the group consisting of phenylene diamine and ditertiarybutyl paracresol prior to warming the oil to above about 40° F.

2. The process according to claim 1 in which the antioxidant is phenylene diamine.

3. The process according to claim 1 in which the antioxidant is ditertiarybutyl paracresol.

## References Cited in the file of this patent

## UNITED STATES PATENTS

|   |           |                |               |
|---|-----------|----------------|---------------|
| 5 | 939,733   | Minor          | Nov. 9, 1909  |
|   | 1,948,281 | Smith          | Feb. 20, 1934 |
|   | 2,202,877 | Stevens et al. | June 4, 1940  |
|   | 2,451,642 | Watson         | Oct. 19, 1948 |
|   | 2,647,868 | Dean           | Aug. 4, 1953  |

## OTHER REFERENCES

10 "Lubrication Engineering," December 1950, pages 263-266.